

# UNITED STATES PATENT OFFICE.

WILLIAM VIRGO WILSON, OF JUBILEE STREET, COUNTY OF MIDDLESEX, AND  
JOSEPH STOREY, OF LANCASTER, COUNTY OF LANCASTER, ENGLAND;  
SAID STOREY ASSIGNOR TO SAID WILSON.

## MANUFACTURE OF ARTIFICIAL LEATHER OR LEATHER CLOTH.

SPECIFICATION forming part of Letters Patent No. 352,726, dated November 16, 1886.

(Application filed October 15, 1885. Serial No. 179,976. (Specimens.) Patented in England April 7, 1884, No. 6,051; in France June 25, 1884, No. 162,965; in Belgium June 28, 1884, No. 65,624; in Italy September 30, 1884, XVIII, 17,146, XXXIV, 162, and in Canada April 20, 1885, No. 21,473.

To all whom it may concern:

Be it known that we, WILLIAM VIRGO WILSON, of Jubilee street, in the county of Middlesex, England, color manufacturer, and JOSEPH STOREY, of Lancaster, in the county of Lancaster, England, manufacturing chemist, subjects of the Queen of Great Britain, have invented certain new and useful Improvements in the Manufacture of Artificial Leather or Leather Cloth, (for which Letters Patent from the following countries have been granted, viz: Great Britain, No. 6,051, dated April 7, 1884; France, No. 162,965, dated June 25, 1884; Belgium, No. 65,624, dated June 28, 1884; Italy, 17,146, XVIII and 162, XXXIV, dated September 30, 1884; Canada, No. 21,473, dated April 20, 1885;) and we do hereby declare that the following is a full, clear, and exact description of the invention, which will enable others skilled in the art to which it appertains to make and use the same.

Our invention has for its object the production of a new article of manufacture resembling artificial leather or leather cloth, and being a woven fabric or web coated with a compound consisting, essentially, of a residuum from a solution of nitro-cellulose in acetate of amyl in admixture with oil.

The preferred proportions of the ingredients of the composition from which said residuum is obtained are as follows: acetate of amyl, six hundred parts; nitro cellulose, two hundred parts; castor or linseed oil, three hundred parts; to which may be added two hundred parts of china-clay or other pigment.

The nitro-cellulose is dissolved in or combined with the acetate of amyl, and to this compound, in the form of a stiff paste or dough, the oil and afterward the pigment are added and the whole thoroughly incorporated in a straining or masticating machine or passed

through grinding-rolls, to which heat may be applied with advantage, whereby a homogeneous mass is produced, which is then spread upon the fabric or web by means of a machine similar to those commonly used for spreading india-rubber and gutta-percha upon fabrics.

We are aware of the patent to Lewthwaite, dated May 17, 1870, No. 103,209, in which a fabric is coated with parkesine or xylonite. This compound is, however, of altogether different physical and chemical characteristics both in respect to the solid or pigmentary ingredients and also the solvents. In our product the coating is composed of mononitro-cellulose and vegetable oil and coloring-matter as pigments and acetate of amyl as the solvent, and great advantages are obtained both as regards the quality of the finished article and the speed of its production, which is due to the nature of its composition.

We claim—

As a new article of manufacture, a fabric coated with the residuum from a solution of mononitro cellulose in acetate of amyl in admixture with oil and a pigmentary matter, as described.

Dated this 9th day of May, 1885.

WILLIAM VIRGO WILSON.

JOSEPH STOREY.

Witnesses to the signature of William Virgo Wilson:

W. T. ATKIN,  
East London Color Works, Jubilee Street, Mercantile Clerk.

E. G. WEIGHTMAN,  
75 Bramcote Road, Rotherhithe New Road, S. E., Mercantile Clerk.

Witnesses to the signature of Joseph Storey:

ROBT. HALE,  
JAMES W. MARSHALL,  
Both Solicitors, Lancaster.